

# UNITED STATES PATENT OFFICE.

CHARLES L. GABRIEL, OF NEW YORK, N. Y.

## MATCH AND METHOD OF MAKING THE SAME.

1,147,159.

Specification of Letters Patent. Patented July 20, 1915.

No Drawing.

Application filed October 11, 1913. Serial No. 794,556.

To all whom it may concern:

Be it known that I, CHARLES L. GABRIEL, a citizen of the United States, residing at the city of New York, borough of Brooklyn, 5 Kings county, and State of New York, have invented certain new and useful Improvements in Matches and Methods of Making the Same, of which the following is a full, clear, and exact specification.

10 My invention relates to an improvement in matches and method of making the same, and it has for its object more particularly to provide a simple, effective and economical method of treating the match splint in order 15 to render it non-glowing after the flame has been extinguished.

To the attainment of the aforesaid object and end, my invention consists in the steps or treatment, constituting my invention, 20 hereinafter more fully described and then pointed out in the claims.

Matches as ordinarily made consist of thin sticks or splints of soft wood which are first impregnated with an agent such as paraffin 25 in order to render the splint more readily ignitable, whereupon the splint is dipped into a suitable mixture composed essentially of phosphorus, which when dry forms a combustible head on the end of the splint.

30 The making of matches according to the method briefly above outlined results in the production of a match which will, after it has been ignited and its flame subsequently extinguished be provided with a splint which 35 will glow or remain incandescent for an appreciable period or time. This afterglow of the burnt or charred splint is frequently the cause of fire and other accidents, which might be prevented if the afterglow or in-

40 candescent state of the splint did not continue after the flame is extinguished. In order, therefore, to prevent this afterglow, and to render the match more safe for use, I treat the splint prior to its impregnation

45 with paraffin, with an agent which will render the splint non-glowing, i. e., will cause the match to become completely extinguished and free from all afterglow or incandescence the instant the flame is extinguished. To

50 the attainment of this result, I impregnate the match splint, before the same has been impregnated with paraffin, with a solution consisting of a liquid hydrocarbon combined with an aromatic oil; or with a fatty acid; 55 or with benzol, toluol, xylol, or similar

bodies. This solution serves as a solvent in which I dissolve one per cent. (1%) of trichlorid of phosphorus or pentachlorid of phosphorus.

By preference I form the impregnating 60 solution by mixing about two pounds of benzol with about one pound of trichlorid of phosphorus, and then bringing the same to a temperature of about 78° C., and maintaining the same at said temperature for 65 fifteen to twenty minutes. Hereupon I allow the mixture to cool, and when the same has cooled down to about atmospheric temperature I add the same to about one hundred pounds of kerosene oil. 70

If the impregnating is to be done with paraffin as a vehicle, instead of with liquid petroleum, the solution should be heated to about the melting point of paraffin, i. e. 100° C. in order to render the same fluid. 75

It is to be noted particularly that instead of combining an aromatic hydrocarbon with kerosene or petroleum oil to form a solvent, I may substitute instead of the aromatic hydrocarbon one of the fatty acid compounds, or any similar body. Further it is to be noted that I may cause impregnating material, viz: the trichlorid or pentachlorid of phosphorus to react on the solvent, viz: 80 and enter into chemical combination therewith, thus changing the character of the solvent, or I may cause the impregnating material to react with the linseed oil, fatty acid, benzol, toluol, or xylol, and then add the resultant compound to the solvent as 85 above described.

Having thus described my said invention, what I claim and desire to secure by Letters Patent is:

1. The method of preparing match splints 95 which consists in impregnating the same with a solution comprising a phosphorus chlorid, a solvent therefor, and a vehicle, substantially as specified.

2. The method of preparing match splints 100 which consists in impregnating the same with a solution comprising a phosphorus chlorid, a solvent therefor and a liquid hydrocarbon, substantially as specified.

3. The method of preparing match splints 105 which consists in impregnating the same with a solution consisting of trichlorid of phosphorus dissolved in a liquid hydrocarbon, substantially as specified.

4. The method of preparing match splints 110

which consists in impregnating the same with a solution consisting of trichlorid of phosphorus dissolved in benzol, and mixed with petroleum, substantially as specified.

5 5. The method of preparing match splints which consists in impregnating the same with a solution consisting of trichlorid of phosphorus dissolved in benzol and mixed with a petroleum derivative, substantially as 10 specified.

6. The method of preparing match splints which consists in impregnating the same with a solution composed of trichlorid of phosphorus about one pound; benzol about 15 two pounds, mixed with kerosene about one hundred pounds, substantially as specified.

7. A match splint formed of a suitable substance impregnated with a solution consisting of trichlorid of phosphorus dissolved 20 in benzol, and a liquid hydrocarbon, substantially as specified.

8. A match splint formed of a suitable

substance impregnated with a solution consisting of trichlorid of phosphorus dissolved in benzol and mixed with petroleum, substantially as specified. 25

9. A match splint formed of a suitable substance impregnated with a solution consisting of trichlorid of phosphorus, dissolved in benzol and mixed with kerosene, 30 substantially as specified.

10. A match splint formed of a suitable substance impregnated with a solution consisting of trichlorid of phosphorus, about one pound; benzol, about two pounds mixed 35 with kerosene, about one hundred pounds, substantially as specified.

Signed at the city of New York, the 25th day of September, one thousand nine hundred and thirteen.

CHARLES L. GABRIEL.

Witnesses:

Wm. M. SILVERMAN,  
DOROTHY SCHONHAUS.